

# United States Patent Office

3,497,334  
Patented Feb. 24, 1970

1

3,497,334

LIQUID HYDROCARBON COMBUSTION FUELS  
Paul Y. C. Gee, Woodbury, and Harry J. Andress, Jr.,  
Pitman, N.J., assignors to Mobil Oil Corporation, a cor-  
poration of New York  
No Drawing. Filed Dec. 16, 1963, Ser. No. 330,590  
Int. Cl. C10I 1/22; C07d 49/00; C07c 103/14  
U.S. Cl. 44—71

24 Claims

This invention relates to liquid hydrocarbon combustion fuels. More particularly, the invention relates to liquid hydrocarbon combustion fuels that are stabilized against screen-clogging, sediment formation, oxidation and metal activity, and to novel additive compositions therefor.

As is well known to those familiar with the art, liquid hydrocarbon combustion fuels, such as fuel oils and gasolines, tend to exhibit certain deleterious characteristics, either after long periods of storage, or under the conditions of operational use. Thus, for example, fuel oils have been found to be unstable in high temperature environment and tend to foul heat-exchange tubes and to cause clogging of screens and plugging of tubes. Sediment formation is another factor often encountered. In gasolines, as well as in fuel oils, oxidation and the effect of metal activity are also undesirable phenomena that are sought to be eliminated. Accordingly, a means for stabilizing such fuels and protecting them against sediment formation, screen clogging, oxidation and metal activity, is highly desirable.

It is, therefore, an object of the present invention to provide improved liquid hydrocarbon combustion fuels.

Another object of the invention is to provide improved liquid hydrocarbon combustion fuels and means for protecting them, which are effective sediment stabilizers, antioxidants and metal deactivators.

Other objects and advantages inherent in the invention will become apparent to those skilled in the art from the following description.

In accordance with the present invention, as more fully hereinafter discussed, it has been found that the above objects can be attained by the addition of small amounts of additive compositions comprising the product obtained by reacting an alkenyl succinic acid anhydride with a polyamine having the formula  $H_2N(-R-NH)_n-H$ , wherein R is selected from the group consisting of ethylene and propylene and n is an integer varying from 1 to 6, and salicylaldehyde. As will become hereinafter apparent, these additive compositions are particularly effective as sediment stabilizers in fuel oils and as antioxidants and metal deactivators in both fuel oils and gasolines.

In the novel additive compositions of the present invention any alkenyl succinic acid anhydride, or the corresponding acid, is utilizable. The general structural formulae of these compounds are:



wherein R is an alkenyl radical. The alkenyl radical can be straight-chain or branched-chain; and it can be saturated at the point of unsaturation by the addition of a substance which adds to olefinic double bonds, such as hydrogen, sulfur, bromine, chlorine, or iodine. It is obvious, of course, that there must be at least two carbon

atoms in the alkenyl radical, but there is no real upper limit to the number of carbon atoms therein. The alkenyl succinic acid anhydrides and the alkenyl succinic acids are interchangeable for the purposes of the present invention. Accordingly, when the term "alkenyl succinic acid anhydride," is used herein, it must be clearly understood that it embraces the alkenyl succinic acids as well as their anhydrides, and the derivatives thereof in which the olefinic double bond has been saturated, as set forth hereinbefore. Non-limiting examples of the alkenyl succinic acid anhydride component are ethenyl succinic acid anhydride; ethenyl succinic acid; ethyl succinic acid anhydride; propenyl succinic acid anhydride; sulfurized propenyl succinic acid anhydride; butenyl succinic acid; 2-methylbutenyl succinic acid anhydride; 1,2-dichloropentenyl succinic acid anhydride; hexenyl succinic acid anhydride; hexyl succinic acid; sulfurized 3-methylpentenyl succinic acid anhydride; 2,3-dimethylbutenyl succinic acid anhydride; 3,3-dimethylbutenyl succinic acid; 1,2-dibromo-2-ethylbutyl succinic acid; heptenyl succinic acid anhydride; 1,2-diiodooctyl succinic acid; octenyl succinic acid anhydride; diisobutetyl succinic acid anhydride; 2-methylheptenyl succinic acid anhydride; 4-ethylhexenyl succinic acid; 2-isopropylphentenyl succinic acid anhydride; nonenyl succinic acid anhydride; 2-propylhexenyl succinic acid anhydride; decenyl succinic acid; decenyl succinic acid anhydride; 5-methyl-2-isopropyl-hexenyl succinic acid anhydride; 1,2-dibromo-2-ethyloctenyl succinic acid anhydride; decyl succinic acid anhydride; undecenyl succinic acid anhydride; 1,2-dichloroundecyl succinic acid; 3-ethyl-2-t-butyl-pentenyl succinic acid anhydride; tetrapropenyl succinic acid anhydride; tetrapropenyl succinic acid; triisobutetyl succinic acid anhydride; 2-propyl-nonyl succinic acid anhydride; 2-butyloctenyl succinic acid anhydride; tridecenyl succinic acid anhydride; hexadecenyl succinic acid anhydride; sulfurized octadecenyl succinic acid; octadecenyl succinic acid anhydride; 1,2-dibromo-2-methylpentadecenyl succinic acid anhydride; 8-propylpentadecyl succinic acid anhydride; eicosenyl succinic acid anhydride; 1,2-dichloro-2-methylnonadecenyl succinic acid anhydride; 2-octyldodecenyl succinic acid; 1,2-diiodotetraacosenyl succinic acid anhydride; hexacosenyl succinic acid; hexacosenyl succinic acid anhydride; and hentriacontenyl succinic acid anhydride. In general, alkenyl succinic acid anhydrides having from about 8 to about 35, and preferably, from about 9 to about 18 carbon atoms in the alkenyl group thereof, are most advantageously employed in the novel additive compositions. Methods for preparing the alkenyl succinic acid anhydrides are well known to those familiar with the art, the most feasible method comprising the reaction of an olefin with maleic acid anhydride. A more detailed description of the alkenyl succinic acid anhydrides suitable for use in the additive compositions of the present invention and their preparation, is disclosed in Patent No. 2,638,450, issued May 12, 1953.

The polyamine reactant, employed with the alkenyl succinic acid anhydride and the salicylaldehyde reactants, as indicated above, has the formula  $H_2N(-R-NH)_n-H$ , wherein R is selected from the group consisting of ethylene and propylene and n is an integer varying from 1 to 6. Examples of the polyamine reactant are ethylenediamine, propylenediamine, diethylenetriamine, triethylenetetramine, tetraethylenepentamine, dipropylenetriamine, and aminopropyl substituted alkylamines. The aminopropyl substituted alkyl amines have the general formula



wherein R represents a mixture of alkyl groups derived from a fatty acid.

The polyamine reactant is preferably employed in an amount from about 1 to about 2 moles per mole of alkenyl succinic acid anhydride, and the salicylaldehyde reactant is preferably employed in an amount from about 1 to about 10 moles per mole of alkenyl succinic acid anhydride, in the additive composition.

The additive composition, i.e. the aforementioned reaction product, is added to the fuel in a small amount to attain the objects hereinbefore discussed. In general, the additive composition may vary from about 1 to about 200, and, preferably, from about 1 to about 25 pounds per thousand barrels of fuel; or, in corresponding terms of percent, by weight, the concentration of additive composition may vary from about 0.00025 to about 0.1, and, preferably, from about 0.00025 to about 0.01 percent, by weight, of the fuel.

The following examples and comparative data are intended to illustrate the novel additive compositions of the present invention and to demonstrate their effectiveness in improving the properties of liquid hydrocarbon combustion fuels. It will be understood, of course, that it is not intended the invention be limited to the particular compositions shown or to the operations or manipulations involved. Various other additive compositions, and other fuels, can be utilized, as those skilled in the art will readily appreciate.

#### EXAMPLE 1

40 grams ( $\frac{2}{3}$  mole) of ethylenediamine were gradually added at room temperature with stirring to 88.7 grams ( $\frac{1}{3}$  mole) of tetrapropenylsuccinic acid anhydride, which were diluted with 192 grams of xylene and 100 cc. of benzene. The reaction was exothermic and the temperature rose rapidly to  $65^{\circ}$  C. At the completion of the addition, the mixture was stirred at  $75$ – $80^{\circ}$  C. for a period of 30 minutes. To this reaction mixture were then added 81.3 grams ( $\frac{2}{3}$  mole) of salicylaldehyde at room temperature with stirring. The resulting mixture was then refluxed at  $95$ – $100^{\circ}$  C. for a period of 3 hours, and then at  $130^{\circ}$  C. until water could no longer be collected (i.e., after a period of about 2 hours). The amount of water collected was 20 cc., (theory 18 cc.). The reaction product obtained, was found to contain approximately 50 percent, by weight, xylene, and was clear and fluid at  $70^{\circ}$  C. Upon analysis, this reaction product showed a nitrogen content of 4.71 percent, as against an estimated 4.87 percent, by weight.

#### EXAMPLE 2

49.3 grams ( $\frac{2}{3}$  mole), equivalent to 61.6 grams of 80 percent propylenediamine, was gradually added to a mixture of 88.7 grams ( $\frac{1}{3}$  mole) of tetrapropenylsuccinic acid anhydride and 201 grams of xylene at room temperature, with stirring. This mixture was then stirred at  $95^{\circ}$  C. for a period of two hours. To this reaction mixture were then gradually added 81.3 grams ( $\frac{2}{3}$  mole) of salicylaldehyde at room temperature, with stirring. The resulting mixture was then slowly heated to the reflux temperature ( $145^{\circ}$  C.), and maintained at this temperature until water could no longer be collected (i.e., after a period of about 3 hours). The amount of water collected was 29 cc., (theory 30 cc.). The reaction product obtained was filtered through clay, and the final product obtained was found to contain approximately 50 percent, by weight, xylene, and was dark brown in color, clear and fluid at room temperature. Upon analysis this reaction product showed a nitrogen content of 4.9 percent, as against an estimated 4.5 percent, by weight.

#### EXAMPLE 3

51.5 grams (0.5 mole) of diethylenetriamine were gradually added to a mixture of 66.5 grams (0.25 mole) of tetrapropenylsuccinic acid anhydride and 165 grams of xylene, as a diluent, at room temperature with stirring, followed by the addition of 61 grams (0.5 mole) of salicylaldehyde, diluted with 50 cc. of benzene. The mixture was gradually heated to reflux at  $135^{\circ}$  C., and maintained

at this temperature until water could no longer be collected (i.e., after a period of about 3 hours). The amount of water collected was 15 cc., (theory 13.5 cc.). The reaction product was filtered through clay, and the final product obtained was found to contain approximately 50 percent, by weight, xylene, and was clear and fluid at room temperature. Upon analysis this reaction product showed a nitrogen content of 5.87 percent, as against an estimated 6.5 percent, by weight.

#### EXAMPLE 4

73 grams (0.5 mole) of triethylenetetramine were gradually added at room temperature, with stirring, to a mixture of 66.5 grams (0.25 mole) of tetrapropenylsuccinic acid anhydride and 187 grams of xylene, followed by the addition of 61 grams (0.5 mole) of salicylaldehyde diluted with 50 cc. of benzene. This mixture was gradually heated to reflux at  $135^{\circ}$  C., and was maintained at this temperature until water could no longer be collected (i.e., after a period of about 2 hours). The amount of water collected was 15 cc., (theory 13.5 cc.). The resulting reaction product was then filtered through clay, and the final product obtained was found to contain approximately 50 percent, by weight, of xylene and was clear and fluid at room temperature. Upon analysis, this final reaction product showed a nitrogen content of 7.23 percent, as against an estimated 7.7 percent, by weight.

#### EXAMPLE 5

94.5 grams (0.5 mole) of tetraethylenepentamine were gradually added at room temperature, with stirring, to a mixture of 66.5 grams (0.25 mole) of tetrapropenylsuccinic acid anhydride and 208 grams of xylene, followed by the addition of 61 grams (0.5 mole) of salicylaldehyde, diluted with 50 cc. of benzene. The mixture was gradually heated to reflux at  $135^{\circ}$  C., and was maintained at this temperature until water could no longer be collected (i.e., after a period of about 3 hours). The amount of water collected was 15 cc., (theory 13.5 cc.). The reaction product obtained was filtered through clay, and the final product obtained was found to contain approximately 50 percent, by weight, xylene, and was clear and fluid at room temperature. Upon analysis, this reaction product showed a nitrogen content of 8.41 percent, as against an estimated 8.4 percent, by weight.

#### EXAMPLE 6

61 grams (0.5 mole) of salicylaldehyde were gradually added to a mixture of 160 grams (0.5 mole) of an aminopropyl substituted alkyl amine having the formula



and 256 grams of xylene at room temperature, with stirring. At the end of the addition, the resulting mixture was gradually heated to reflux at  $145^{\circ}$  C., and was maintained at this temperature until water could no longer be collected (i.e., after a period of about 2 hours). The amount of water collected was 10 cc., (theory 9 cc.). To this reaction mixture were then added 66.5 grams (0.25 mole) of tetrapropenylsuccinic acid anhydride at room temperature. This resulting mixture was then refluxed at  $145^{\circ}$  C. until water could no longer be collected (i.e., after a period of about 3 hours). The amount of water collected was 4.5 cc. (theory 4.5 cc.). The resulting reaction product was filtered through clay, and the final product obtained was found to contain approximately 50 percent, by weight, of xylene and was dark red in color, clear and fluid at room temperature. Upon analysis, this final reaction product showed a nitrogen content of 2.93 percent, as against an estimated 2.74 percent, by weight.

#### EXAMPLE 7

30.5 grams (0.25 mole) of salicylaldehyde, diluted with 50 cc. of benzene, were gradually added at room temperature, with stirring, to a mixture of 100 grams (0.25 mole) of an aminopropyl substituted alkyl amine having

the formula  $\text{RNHCH}_2\text{CH}_2\text{CH}_2\text{NH}_2$  and 157 grams of xylene. At the end of this addition, the resulting mixture was gradually heated to reflux at a temperature of  $126^\circ\text{ C.}$ , and maintained at this temperature until water could no longer be collected (i.e., after a period of about 2 hours). The amount of water collected was 5.5 cc., (theory 4.5 cc.). To this reaction mixture were then added 33.25 grams (0.125 mole) of tetrapropenylsuccinic acid anhydride at room temperature. This resulting mixture was then refluxed at  $140^\circ\text{ C.}$  until water could no longer be collected (i.e., after a period of about 2 hours). The amount of water collected was 2.5 cc. (theory 2.25 cc.). The resulting reaction product was filtered through clay, and the final product obtained was found to contain approximately 50 percent, by weight, of xylene, and was dark red in color, clear and fluid at room temperature. Upon analysis, this reaction product showed a nitrogen content of 2.57 percent, as against an estimated 2.22 percent, by weight.

## EXAMPLE 8

49.3 grams ( $\frac{2}{3}$  mole), equivalent to 54.8 grams of 90 percent propylenediamine, was gradually added at room temperature, with stirring, to a mixture of 75 grams ( $\frac{1}{3}$  mole) of nonenylsuccinic acid anhydride and 187 grams of xylene, followed by the addition of 81.3 grams ( $\frac{2}{3}$  mole) of salicylaldehyde. The resulting mixture was slowly heated to reflux at a temperature of  $142\text{--}145^\circ\text{ C.}$ , and maintained at this temperature until water could no longer be collected (i.e., after a period of about 3 hours). The amount of water collected was 23 cc. (theory 23.5 cc.). The reaction product was then filtered through clay, and the final product obtained was found to contain approximately 50 percent, by weight, of xylene, and was clear and fluid at room temperature. Upon analysis, this final reaction product showed a nitrogen content of 6.02 percent, as against an estimated 5.0 percent, by weight.

## EXAMPLE 9

37 grams (0.5 mole), equivalent to 41 grams of 90 percent propylenediamine, were gradually added at room temperature, with stirring, to a mixture of 62.5 grams (0.25 mole) of octadecenyl succinic acid anhydride and 147 grams of xylene, followed by the addition of 61 grams (0.5 mole) of salicylaldehyde. The resulting mixture was then slowly heated to reflux temperature at  $142\text{--}145^\circ\text{ C.}$ , and maintained at that temperature until water could no longer be collected (i.e., after a period of about 3 hours). The amount of water collected was 17.5 cc. (theory 17.5 cc.). The resulting reaction product was then filtered through clay, and the final product obtained was found to contain approximately 50 percent, by weight, of xylene, and was clear and fluid at room temperature. Upon analysis, this reaction product showed a nitrogen content of 4.67 percent, as against 4.71 percent, by weight.

The additive compositions of the present invention impart valuable properties, as hereinbefore indicated, to liquid hydrocarbon combustion fuels, including the distillate fuels, i.e., gasolines and fuel oils. Accordingly, the fuel oils that may be improved in accordance with the present invention are hydrocarbon fractions having an initial boiling point of at least about  $100^\circ\text{ F.}$  and an end-boiling point no higher than about  $750^\circ\text{ F.}$ , and boiling substantially continuously throughout their distillation range. Such fuel oils are generally known as distillate fuel oils. It is to be understood, however, that this term is not restricted to straight-run distillate fractions. The distillate fuel oils can be straight-run distillate fuel oils, catalytically or thermally cracked (including hydrocracked) distillate fuel oils, or mixtures of straight-run distillate fuel oils, naphthas and the like, with cracked distillate stocks. Moreover, such fuel oils can be treated in accordance with well known commercial methods, such as, acid or caustic treatment, hydrogenation, solvent refining, clay treatment, etc.

The distillate fuel oils are characterized by their rela-

tively low viscosities, pour points, and the like. The principal property which characterizes the contemplated hydrocarbons, however, is the distillation range. As mentioned hereinbefore, this range will lie between about  $100^\circ\text{ F.}$  and about  $750^\circ\text{ F.}$  Obviously, the distillation range of each individual fuel oil will cover a narrower boiling range falling, nevertheless, within the above-specified limits. Likewise, each fuel oil will boil substantially continuously throughout its distillation range.

Particularly contemplated among the fuel oils are Nos. 1, 2, and 3 fuel oils used in heating and as diesel fuel oils, and the jet combustion fuels. The domestic fuel oils generally conform to the specifications set forth in A.S.T.M. Specifications D396-48T. Specifications for diesel fuels are defined in A.S.T.M. Specification D975-48T. Typical jet fuels are defined in Military Specification MIL-F-5624B.

The gasolines that are improved by the additive compositions of this invention, are mixtures of hydrocarbons having an initial boiling point falling between about  $75^\circ\text{ F.}$  and about  $135^\circ\text{ F.}$  and an end-boiling point falling between about  $250^\circ\text{ F.}$  and about  $450^\circ\text{ F.}$  As is well known to the art, motor gasoline can be straight run gasoline or, as is more usual, it can be a blend of two or more cuts or materials including straight run stock, catalytic or thermal reformate, cracked stock, alkylated natural gasoline, and aromatic hydrocarbons.

## Screen clogging

The anti-screen clogging characteristics of a fuel oil are determined as follows: the test is conducted using a Sunstrand V3 or S1 home fuel oil burner pump with a self-contained 100-mesh Monel metal screen. About 0.05 percent, by weight, of naturally-formed fuel oil sediment, composed of fuel oil, water, dirt, rust, and organic sludge is mixed with 10 liters of the fuel oil. The mixture is circulated by the pump through the screen for 6 hours. Then, the sludge deposit on the screen is washed off with normal pentane and filtered through a tared Gooch crucible. After drying, the material in the Gooch crucible is washed with a 50-50 (volume) acetone-methanol mixture. The total organic sediment is obtained by evaporating the pentane and the acetone-methanol filtrates. Drying and weighing the Gooch crucible yields the amount of inorganic sediment. The sum of the organic and inorganic deposits on the screen can be reported in milligrams recovered or converted into percent screen clogging.

The uninhibited test fuel oil was a blend of 60 percent distillate stock obtained from continuous catalytic cracking and 40 percent straight-run distillate stock, having a boiling range of, approximately, from about  $320^\circ\text{ F.}$  to about  $640^\circ\text{ F.}$ , and representing a typical No. 2 fuel oil.

Blends of the additives of the examples were prepared in the aforescribed test fuel oil and subjected to the screen clogging test. Results are set forth in Table I.

TABLE I.—FUEL OIL SCREEN CLOGGING

| Additive of Example                   | Cone <sup>n</sup> ,<br>lbs./1,000<br>bbls. | Screen<br>Clogging,<br>Percent |
|---------------------------------------|--------------------------------------------|--------------------------------|
| Uninhibited fuel blend-----           | 0                                          | 100                            |
| Uninhibited fuel blend+Example 1----- | 50                                         | 30                             |
| Uninhibited fuel blend+Example 2----- | 25                                         | 8                              |
| Uninhibited fuel blend+Example 3----- | 25                                         | 20                             |
| Uninhibited fuel blend+Example 5----- | 25                                         | 25                             |
| Uninhibited fuel blend+Example 6----- | 10                                         | 5                              |
| Uninhibited fuel blend+Example 7----- | 25                                         | 10                             |
| Uninhibited fuel blend+Example 8----- | 25                                         | 63                             |
| Uninhibited fuel blend+Example 9----- | 25                                         | 5                              |

## Sedimentation

The test used to determine the sedimentation characteristics of the fuel oils is the  $110^\circ\text{ F.}$  storage test. In this test, a 500-milliliter sample of the fuel oil under test is placed in a convected oven maintained at  $110^\circ\text{ F.}$

for a period of 12 weeks. Then, the sample is removed from the oven and cooled. The cooled sample is filtered through a tared asbestos filter (Gooch crucible) to remove insoluble matter. The weight of such matter in milligrams is reported as the amount of sediment. A sample of the blank, uninhibited oil is run along with a fuel oil blend under test. The effectiveness of a fuel oil containing an inhibitor is determined by comparing the weight of sediment formed in the inhibited oil with that formed in the uninhibited oil.

Additives described in the example were blended in the aforementioned test fuel oil and the blends were subjected to the 110° F. storage test. The test results comparing the blended fuels and uninhibited fuels are set forth in Table II.

TABLE II.—FUEL OIL 110° F. STORAGE TEST—12 WEEKS

| Additive of Example              | Cone'n.,<br>1,000 bbls. | Sediment<br>mg./liter |
|----------------------------------|-------------------------|-----------------------|
| Uninhibited fuel blend           | 0                       | 77                    |
| Uninhibited fuel blend+Example 2 | 10                      | 62                    |
| Uninhibited fuel blend<br>Do     | 0                       | 8                     |
| Uninhibited fuel blend+Example 6 | 25                      | 3                     |
| Uninhibited fuel blend           | 0                       | 8                     |
| Uninhibited fuel blend+Example 7 | 25                      | 4                     |
| Uninhibited fuel blend           | 0                       | 69                    |
| Uninhibited fuel blend+Example 8 | 25                      | 54                    |
| Uninhibited fuel blend           | 0                       | 8                     |
| Uninhibited fuel blend+Example 9 | 10                      | 3                     |

30

#### Gasoline storage test

This test was used to determine the quantity of gum increase in both a gasoline blend comprising 100 percent catalytically cracked components and containing 3 cc. tetraethyl lead (TEL) per gallon, and boiling within a 100–400° F. boiling range, and the same gasoline blend containing, also, the additive compositions of the examples. After being maintained at 110° F. for a period of 16 weeks, the amount of gum increase was determined according to A.S.T.M. Test D381. The test results comparing the uninhibited gasolines and the same gasolines containing the additive compositions of the examples, are set forth in Table III.

TABLE III.—GASOLINE STORAGE TEST

| Additive of Example                               | Weeks<br>at<br>110° F. | Cone'n.,<br>lbs./1,000<br>bbls. | ATSM<br>Gum<br>Increase,<br>mg./100 ml. |
|---------------------------------------------------|------------------------|---------------------------------|-----------------------------------------|
| Uninhibited gasoline+3 cc. TEL/gal.               | 16                     | 0                               | 42.7                                    |
| Uninhibited gasoline+3 cc. TEL/<br>gal.+Example 1 | 16                     | 10                              | 1.9                                     |
| Uninhibited gasoline+3 cc. TEL/gal.               | 16                     | 0                               | 42.7                                    |
| Uninhibited gasoline+3 cc. TEL/<br>gal.+Example 2 | 16                     | 5                               | 1.7                                     |
| Uninhibited gasoline+3 cc. TEL/gal.               | 16                     | 0                               | 19.7                                    |
| Uninhibited gasoline+3 cc. TEL/<br>gal.+Example 3 | 16                     | 10                              | 2.5                                     |
| Uninhibited gasoline+3 cc. TEL/gal.               | 16                     | 0                               | 19.7                                    |
| Uninhibited gasoline+3 cc. TEL/<br>gal.+Example 4 | 16                     | 10                              | 1.4                                     |
| Uninhibited gasoline+3 cc. TEL/gal.               | 16                     | 0                               | 2.6                                     |
| Uninhibited gasoline+3 cc. TEL/<br>gal.+Example 5 | 16                     | 5                               | 1.6                                     |
| Uninhibited gasoline+3 cc. TEL/gal.               | 16                     | 0                               | 1.4                                     |
| Uninhibited gasoline+3 cc. TEL/<br>gal.+Example 8 | 16                     | 2                               | 0.5                                     |

#### Gasoline storage test with copper

The same test procedure, as described in the Gasoline Storage Test, (supra), was employed, with the same gasoline blends containing 3 cc. tetraethyl lead (TEL) per gallon, and also including 0.2 mg. copper naphthenate per liter, as a metal catalyst. The test results comparing the uninhibited gasolines and the same gasolines

70  
75

containing the additive compositions of the examples, are set forth in Table IV.

TABLE IV.—GASOLINE STORAGE TEST

| Additive of Example                                                               | Weeks<br>at<br>110° F. | Cone'n.,<br>lbs./1,000<br>bbls. | ATSM<br>Gum<br>Increase,<br>mg./100 ml. |
|-----------------------------------------------------------------------------------|------------------------|---------------------------------|-----------------------------------------|
| Uninhibited gasoline+3 cc. TEL/<br>gal.+0.2 mg Cu naphthenate/liter               | 16                     | 0                               | 75.0                                    |
| Uninhibited gasoline+3 cc. TEL/<br>gal.+0.2 mg Cu naphthenate/liter+<br>Example   | 16                     | 5                               | 5.1                                     |
| Uninhibited gasoline+3 cc. TEL/<br>gal.+0.2 mg Cu naphthenate/liter               | 16                     | 0                               | 75.0                                    |
| Uninhibited gasoline+3 cc. TEL/<br>gal.+0.2 mg Cu naphthenate/liter+<br>Example 2 | 16                     | 3                               | 3.9                                     |
| Uninhibited gasoline+3 cc. TEL/<br>gal.+0.2 mg Cu naphthenate/liter               | 16                     | 0                               | 21.5                                    |
| Uninhibited gasoline+3 cc. TEL/<br>gal.+0.2 mg Cu naphthenate/liter+<br>Example 3 | 16                     | 10                              | 12.6                                    |
| Uninhibited gasoline+3 cc. TEL/<br>gal.+0.2 mg Cu naphthenate/liter               | 16                     | 0                               | 26.5                                    |
| Uninhibited gasoline+3 cc. TEL/<br>gal.+0.2 mg Cu naphthenate/liter+<br>Example 4 | 16                     | 10                              | 8.1                                     |
| Uninhibited gasoline+3 cc. TEL/<br>gal.+0.2 mg Cu naphthenate/liter               | 16                     | 0                               | 21.5                                    |
| Uninhibited gasoline+3 cc. TEL/<br>gal.+0.2 mg Cu naphthenate/liter+<br>Example 5 | 16                     | 10                              | 1.5                                     |
| Uninhibited gasoline+3 cc. TEL/<br>gal.+0.2 mg Cu naphthenate/liter               | 16                     | 0                               | 30.4                                    |
| Uninhibited gasoline+3 cc. TEL/<br>gal.+0.2 mg Cu naphthenate/liter+<br>Example 8 | 16                     | 3                               | 3.6                                     |

30

While the present invention has been described with preferred embodiments, it should be understood that modifications and variations thereof may be resorted to without departing from the spirit of the invention as will be obvious to those skilled in the art.

We claim:

1. An additive composition comprising the condensation product obtained by reacting an alkenyl succinic acid or anhydride having from about 8 to about 35 carbon atoms in the alkenyl group thereof, with a polyamine having the formula  $H_2N(-R-NH)_n-H$ , wherein R is selected from the group consisting of ethylene and propylene and n is an integer varying from 1 to 6, and salicylaldehyde.

2. An additive composition comprising the condensation product obtained by reacting an alkenyl succinic acid or anhydride having from about 9 to about 18 carbon atoms in the alkenyl group thereof with a polyamine having the formula  $H_2N(-R-NH)_n-H$ , wherein R is selected from the group consisting of ethylene and propylene and n is an integer varying from 1 to 6, and salicylaldehyde.

3. An additive composition comprising the condensation product obtained by reacting an alkenyl succinic acid or anhydride having from about 8 to about 35 carbon atoms in the alkenyl group thereof with from about 1 to about 2 moles of a polyamine having the formula  $H_2N(-R-NH)_n-H$

wherein R is selected from the group consisting of ethylene and propylene and n is an integer varying from 1 to 6, and from about 1 to about 10 moles salicylaldehyde, per mole of alkenyl succinic acid or anhydride.

4. An additive composition comprising the condensation product obtained by reacting an alkenyl succinic acid or anhydride having from about 9 to about 18 carbon atoms in the alkenyl group thereof with from about 1 to about 2 moles of a polyamine having the formula  $H_2N(-R-NH)_n-H$ , wherein R is selected from the group consisting of ethylene and propylene and n is an integer varying from 1 to 6, and from about 1 to about 10 moles salicylaldehyde, per mole of alkenyl succinic acid anhydride.

5. An additive composition comprising the condensa-

tion product obtained by reacting an alkenyl succinic acid or anhydride having from about 8 to about 35 carbon atoms in the alkenyl group thereof with a polyamine selected from the group consisting of ethylenediamine, propylenediamine, diethylenetriamine, triethylenetetramine, tetraethylenepentamine and aminopropyl substituted alkylamines, and salicylaldehyde.

6. An additive composition comprising the condensation product obtained by reacting an alkenyl succinic acid or anhydride selected from the group consisting of tetrapropenyl succinic acid or anhydride, nonenyl succinic acid anhydride and octadecenyl succinic acid or anhydride with a polyamine having the formula



wherein R is selected from the group consisting of ethylene and propylene and n is an integer varying from 1 to 6, and salicylaldehyde.

7. An additive composition comprising the condensation product obtained by reacting an alkenyl succinic acid or anhydride selected from the group consisting of tetrapropenyl succinic acid or anhydride, nonenyl succinic acid or anhydride and octadecenyl succinic acid or anhydride with from about 1 to about 2 moles of a polyamine selected from the group consisting of ethylenediamine, propylenediamine, diethylenetriamine, triethylenetetramine, tetraethylenepentamine and aminopropyl substituted alkylamines, and from about 1 to about 10 moles salicylaldehyde, per mole of alkenyl succinic acid or anhydride.

8. A liquid hydrocarbon combustion fuel containing from about 1 to about 200 pounds per thousand barrels of fuel of an additive composition comprising the condensation product obtained by reacting an alkenyl succinic acid or anhydride having from about 8 to about 35 carbon atoms in the alkenyl group thereof with from about 1 to about 2 moles of a polyamine having the formula  $\text{H}_2\text{N}(-\text{R}-\text{NH})_n-\text{H}$ , wherein R is selected from the group consisting of ethylene and propylene and n is an integer varying from 1 to 6, and with from about 1 to about 6 moles salicylaldehyde, per mole of alkenyl succinic acid or anhydride.

9. A liquid hydrocarbon combustion fuel containing from about 1 to about 25 pounds per thousand barrels of fuel of an additive composition comprising the condensation product obtained by reacting an alkenyl succinic acid or anhydride having from about 8 to about 35 carbon atoms in the alkenyl group thereof with a polyamine having the formula  $\text{H}_2\text{N}(-\text{R}-\text{NH})_n-\text{H}$ , wherein R is selected from the group consisting of ethylene and propylene and n is an integer varying from 1 to 6, and salicylaldehyde.

10. A liquid hydrocarbon combustion fuel containing from about 1 to about 200 pounds per thousand barrels of fuel of an additive composition comprising the condensation product obtained by reacting an alkenyl succinic acid or anhydride having from about 8 to about 35 carbon atoms in the alkenyl group thereof with a polyamine having the formula  $\text{H}_2\text{N}(-\text{R}-\text{NH})_n-\text{H}$ , wherein R is selected from the group consisting of ethylene and propylene and n is an integer varying from 1 to 6, and salicylaldehyde.

11. A liquid hydrocarbon combustion fuel containing from about 1 to about 200 pounds per thousand barrels of fuel of an additive composition comprising the condensation product obtained by reacting an alkenyl succinic acid or anhydride having from about 9 to about 18 carbon atoms in the alkenyl group thereof with a polyamine having the formula  $\text{H}_2\text{N}(-\text{R}-\text{NH})_n-\text{H}$ , wherein R is selected from the group consisting of ethylene and propylene and n is an integer varying from 1 to 6, and salicylaldehyde.

12. A liquid hydrocarbon combustion fuel containing from about 1 to about 200 pounds per thousand barrels of fuel of an additive composition comprising the con-

densation product obtained by reacting an alkenyl succinic acid or anhydride having from about 8 to about 35 carbon atoms in the alkenyl group thereof with from about 1 to about 2 moles of a polyamine having the formula  $\text{H}_2\text{N}(-\text{R}-\text{NH})_n-\text{H}$ , wherein R is selected from the group consisting of ethylene and propylene and n is an integer varying from 1 to 6, and with from about 1 to about 10 moles salicylaldehyde, per mole of alkenyl succinic acid or anhydride.

13. A liquid hydrocarbon combustion fuel containing from about 1 to about 200 pounds per thousand barrels of fuel of an additive composition comprising the condensation product obtained by reacting an alkenyl succinic acid or anhydride having from about 9 to about 18 carbon atoms in the alkenyl group thereof with from about 1 to about 2 moles of a polyamine having the formula  $\text{H}_2\text{N}(-\text{R}-\text{NH})_n-\text{H}$ , wherein R is selected from the group consisting of ethylene and propylene and n is an integer varying from 1 to 6, and with from about 1 to about 10 moles salicylaldehyde, per mole of alkenyl succinic acid or anhydride.

14. A liquid hydrocarbon combustion fuel containing from about 1 to about 200 pounds per thousand barrels of fuel of an additive composition comprising the condensation product obtained by reacting an alkenyl succinic acid or anhydride having from about 8 to about 35 carbon atoms in the alkenyl group thereof with a polyamine selected from the group consisting of ethylenediamine, propylenediamine, diethylenetriamine, triethylenetetramine, tetraethylenepentamine and aminopropyl substituted alkylamines, and salicylaldehyde.

15. A liquid hydrocarbon combustion fuel containing from 1 to about 200 pounds per thousand barrels of fuel of an additive composition comprising the condensation product obtained by reacting an alkenyl succinic acid or anhydride selected from the group consisting of tetrapropenyl succinic acid or anhydride, nonenyl succinic acid or anhydride and octadecenyl succinic acid or anhydride with a polyamine having the formula



wherein R is selected from the group consisting of ethylene and propylene and n is an integer varying from 1 to 6, and salicylaldehyde.

16. A liquid hydrocarbon combustion fuel containing from 1 to about 200 pounds per thousand barrels of fuel of an additive composition comprising the condensation product obtained by reacting an alkenyl succinic acid or anhydride selected from the group consisting of tetrapropenyl succinic acid or anhydride, nonenyl succinic acid or anhydride and octadecenyl succinic acid or anhydride with from about 1 to about 2 moles of a polyamine selected from the group consisting of ethylenediamine, propylenediamine, diethylenetriamine, triethylenetetramine, tetraethylenepentamine and aminopropyl substituted alkylamines, and from about 1 to about 10 moles salicylaldehyde, per mole of alkenyl succinic acid or anhydride.

17. The reaction product obtained by reacting, under reflux conditions, an acidic substance selected from the group consisting of alkenyl succinic acid and alkenyl succinic anhydride, an amine having the structural formula  $\text{H}_2\text{N}-\text{R}-\text{NH}_2$ , and salicylaldehyde, wherein the alkenyl group contains from about 8 to about 35 carbon atoms and R is selected from the group consisting of ethylene and propylene.

18. The reaction product obtained by reacting, under reflux conditions, an acidic substance selected from the group consisting of alkenyl succinic acid and alkenyl succinic anhydride, an amine having the structural formula  $\text{H}_2\text{N}(-\text{R}-\text{NH})_n-\text{H}$ , and salicylaldehyde, wherein the alkenyl group contains from about 8 to about 35 carbon atoms, R is selected from the group consisting of ethylene and propylene, and n is an integer varying from 2-6.

19. The condensation product obtained by reacting an acidic material selected from the group consisting of

alkenyl succinic acid and alkenyl succinic acid anhydride, an amine having the formula  $H_2N—R—NH_2$ , and salicyl-aldehyde, wherein the alkenyl group contains from about 8 to about 35 carbon atoms and R is selected from the group consisting of ethylene and propylene.

20. The product obtained in accordance with claim 19 wherein said reaction is carried out at a temperature from about 50° C. to about 200° C.

21. The condensation product obtained by reacting an acidic material selected from the group consisting of alkenyl succinic acid and alkenyl succinic acid anhydride, an amine having the formula  $H_2N(—R—NH)_n—H$ , and salicylaldehyde, wherein the alkenyl group contains from about 8 to about 35 carbon atoms, R is selected from the group consisting of ethylene and propylene, and n is an integer varying from 2 to 6.

22. The product obtained in accordance with claim 21 wherein said reaction is carried out at a temperature from about 50° C. to about 200° C.

23. An additive composition comprising the condensation product obtained by reacting about 1 mole of an alkenyl succinic acid or anhydride having from about 8 to about 35 carbon atoms in the alkenyl group thereof, with about 2 moles of a polyamine having the formula

$H_2N(—R—NH)_n—H$ , wherein R is selected from the group consisting of ethylene and propylene and n is an integer varying from 1 to 6, and about 2 moles of salicyl-aldehyde.

24. An additive composition comprising the condensation product obtained by reacting about 1 mole of an alkenyl succinic acid or anhydride having from about 9 to about 18 carbon atoms in the alkenyl group thereof, with about 2 moles of a polyamine having the formula  $H_2N(—R—NH)_n—H$ , wherein R is selected from the group consisting of ethylene and propylene and n is an integer varying from 1 to 6, and about 2 moles of salicyl-aldehyde.

#### References Cited

#### UNITED STATES PATENTS

2,638,450 5/1953 White et al. ----- 44—71 XR  
3,280,034 10/1966 Anzenberger et al. 44—63 XR

PATRICK P. GARVIN, Primary Examiner

U.S. CL. X.R.

44—63; 260—309.7, 534, 557

UNITED STATES PATENT OFFICE  
CERTIFICATE OF CORRECTION

Patent No. 3,497,334 Dated February 24, 1970

Inventor(s) Paul Y.C. Gee and Harry J. Andress, Jr.

It is certified that error appears in the above-identified patent and that said Letters Patent are hereby corrected as shown below:

Column 2, line 34, for "2-butyloctenyl" read --3-butyloctenyl--

Column 2, line 45, for "hentriactontenyl" read --hentriaccontenyl--

SIGNED AND  
SEALED  
JUL 14 1970

(SEAL)

Attest:

Edward M. Fletcher, Jr.

Attesting Officer

WILLIAM E. SCHUYLER, JR.  
Commissioner of Patents